

## UNITED STATES PATENT OFFICE

2,088,417

METHOD OF SECURING LIGHT FASTNESS  
IN TRANSFER COPIESWilliam Hoskins, Jr., La Grange, Ill., assignor  
to Ditto, Incorporated, Chicago, Ill., a corpora-  
tion of West VirginiaNo Drawing. Application May 23, 1936,  
Serial No. 81,514

## 5 Claims. (Cl. 41—31.6)

The present invention relates to improvements in transfer processes for effecting reproduction or transfer of designs, drawings, written and typewritten material and the like from an original or master copy and more particularly to a process of making transfer copies resistant to moisture and of great fastness to light.

In certain of the transfer or reproduction processes of the general character hereinabove referred to a number of copies are produced by transfer either directly or indirectly from a master copy prepared with dyes or coloring matters which are in general of the water and alcohol-soluble type. The most commonly used process of this type is of the hectograph type, wherein the original master sheet, prepared with a suitable dye or coloring matter, is applied to a moistened gelatinous copy mass, the dye or color being largely transferred thereto in reverse, and the copies are then made by applying the copy sheets to the copy mass, each receiving a proportion of the dye or coloring matter to form a copy of the design or writing on the master sheet.

In another reproduction process, the master copy is prepared in reverse by drawing, writing, typing or otherwise producing the design on a master sheet, behind which is a sheet of suitably prepared color-carrying paper with its inked surface facing the master sheet, so that color constituents of the ink on the carbon paper are transferred to the back of the sheet, forming a reverse copy of the design or writing. In preparing copies from this master sheet, the surface of the copy sheet is moistened with a liquid, usually a water-miscible alcoholic liquid, which has a solvent action on the dyes in the ink deposited on the master sheet from the carbon paper, and the moistened copy sheets are applied to the back of the master sheet, a positive image of the original being thereby reproduced upon the copy sheet. In carrying out such processes, aqueous and alcohol soluble dyes are generally used in the color-carrying paper and hence aqueous and alcoholic solvents have been employed to effect the transfer.

In view of the fact that water and alcohol soluble dyes are generally employed in such transfer processes, the character of the colors available for use therein has been seriously limited in many directions; for example, by lack of moisture resistance and by lack of fastness to light. Due to the water-soluble character of the dyes employed, the fingers of the users of the paper have been soiled by contact therewith and

the impressions on the copy sheets have been blurred and smudged on handling.

In accordance with the present invention, the water and alcohol soluble dyes may be advantageously employed in the transfer processes, and increased water resistance and with increased fastness to light may be secured in the copies. Thus the water and alcohol soluble dyes used in the transfer processes, such as methyl violet, crystal violet, fuchsines, magentas, anthraquinones, chrysoidine and the like; the water and alcohol soluble aniline dyes, such as aniline blue, Victoria blue and orange, Nile blue and the like; the water and alcohol soluble azo dyes, such as Congo red, Bismarck brown and the like, may be advantageously used in these processes and copies may be secured on greatly increased fastness to light and water-resistance.

I have found that these desired properties may be advantageously imparted to the water and alcohol soluble dyes used in the transfer processes by contacting the color impressions on the copy sheets with a colloidal material adapted to combine with the colors or dyes to render them substantially water-insoluble and fast to light. Thus I have found, for example, that the highly colloidal clays such as bentonite will react on and with the water and alcohol soluble dyes to increase their fastness to light for a given strength of copy and to render them substantially water resistant. While I am not able to fully explain the reason for this phenomenon, it appears that the dyes are adsorbed by the colloidal particles of the bentonite to form what appears to be a lake having less fugitiveness than the original dye.

In carrying out the present invention, it is essential that the colloidal material such as bentonite be available for contact with the dye transferred to the copy sheet. Thus, the bentonite can be incorporated into the copy paper either with the size or filler compositions; or may be applied to the copy paper having the transfer impression thereon, as a surface wash; or may be incorporated with the paper as part of a surface coating or glaze in preparing it for use in the transfer process. In each of these methods, the bentonite is available to contact the dye on the copy paper and react thereon or therewith to reduce its fugitiveness, increase its water resistance and render it more fast to light.

As illustrative of one method of incorporating the bentonite into the copy paper the following is set forth; however, it is to be understood that

any of the methods set forth above or methods equivalent thereto may be employed with substantially equal advantage.

Thus, with any of the known conventional engine sizes, I incorporate a small quantity of bentonite, say in the order of about 1% to 5% and mix it with the pulp in a beater to uniformly disperse the size and bentonite throughout the pulp. The pulp is then treated in the usual manner to form a sheet suitable for use as copy paper. Or preferably, in connection with a tub size of the usual character, the bentonite may be incorporated to the extent of 1% to 7% and preferably 2% to about 5% or even higher. Of course, if desired, a suspension of bentonite in about these proportions may be used as a separate coating or wash on the copy paper. If desired, small amounts of hygroscopic substances such as glycerine, dextrine, invert sugar or the like in the order of say from 0.1% to 1% may be incorporated with the size composition containing bentonite. These hygroscopic substances prevent the excessive drying out of the sizing composition and thus prevent the loss of bentonite from the paper.

As indicated above, proportions of bentonite greater than 5 to 7% may be employed; however, no enhanced result appears to flow from this increase in the percentage of bentonite. As very little dye is actually transferred onto the copy paper, very little bentonite is actually needed and therefore the amount of bentonite present to react with the transferred dye on the copy paper should be sufficient to produce the desired results. In actual practice, I have found that from 0.5 to 5% of bentonite in the size or surface wash is sufficient.

The copy paper or sheets prepared as hereinbefore described and having bentonite in minute proportions on the copy surface is then employed to receive the copies in the transfer processes of the type hereinbefore referred to, the prepared copy paper being, for example, applied to a hectographic copy mass carrying reverse ink impressions or being moistened and applied to a reverse master copy.

The dye transferred to the copy sheet coats with the bentonite available therein and the dye is thus rendered water-resistant and of increased fastness to light. Copy sheets having a design reproduced thereon according to my process can be readily handled without soiling the fingers of the users and without smudging and blurring of the impressions, and do not rapidly fade or lose strength or brilliance on exposure to light as with copies of similar strength as hitherto produced. Thus, the light-fastness of the copies made in accordance with the present invention is found in some cases to be 5 or more times as great as when the same colors are employed with untinted copy papers of the types hitherto in use. Further, the water-fastness of copies made in accordance with the present invention is so greatly increased as to make the copies practically waterproof, as they may be placed in water or under running water without affecting the color or causing bleeding or running of the color.

As pointed out hereinabove, by operating in

accordance with the present invention it is possible to secure, in the copy sheets, colors having characteristics not hitherto secured in such processes employing water-soluble and alcohol-soluble dyes for reproduction purposes, and particularly colors having an increased water resistance and an increased fastness to light.

I claim:

1. The process of reproduction of designs formed from water and alcohol-soluble dyes to render the dyes in the reproduced design moisture resistant and fast to light which comprises applying a copy sheet containing available bentonite on its surface to a surface having a design formed thereon from water or alcohol-soluble dyes and thereby transferring a portion of the dye to said copy sheet to form the design thereon, whereby the dye and bentonite coact to render the dye on the copy sheet moisture resistant and fast to light.

2. The process of reproducing color designs to form color designs having an increased fastness to light which comprises contacting a copy sheet containing available bentonite on its surface to a surface having a design formed thereon from water or alcohol-soluble dyes and thereby transferring a portion of the dye to said copy sheet to form the design thereon, whereby the dye and bentonite coact to render the dye on the copy sheet moisture resistant and fast to light.

3. The process of reproducing color designs to form color designs having an increased fastness to light which comprises contacting a copy sheet containing a small quantity of bentonite uniformly applied on the surface of the sheet to a surface having a design formed thereon from water or alcohol-soluble dyes and thereby transferring a portion of the dye to said copy sheet to form the design thereon, whereby the dye and bentonite coact to render the dye on the copy sheet moisture resistant and fast to light.

4. The process of reproducing color designs to form color designs having an increased fastness to light which comprises applying to a master sheet a water or alcohol soluble dye to form a design in reverse, moistening a copy sheet containing bentonite with a solvent and applying the moistened copy sheet to the side of the master sheet bearing said dye, thereby transferring a portion of the dye to said copy sheet to form the design thereon, whereby the dye and bentonite coact to render the dye on the copy sheet moisture resistant and fast to light.

5. The process of reproducing color designs in a hectograph process to form color designs having an increased fastness to light which comprises applying to a sheet a water or alcohol soluble dye to form a design thereon, contacting the design on said sheet with a copy pad to transfer the design in reverse to said pad, and contacting a copy sheet containing available bentonite on its surface with the copy pad to transfer the design to said copy sheet, whereby the dye and bentonite coact to render the dye on the copy sheet moisture resistant and fast to light.

WILLIAM HOSKINS, JR.